# EUROPEAN PATENT SPECIFICATION

(11) **EP 1 474 565 B1**
(45) Date of publication and mention of the grant of the patent: **26.03.2008**
(21) Application number: 03739784.1
(22) Date of filing: 12.02.2003
(51) Int. Cl.: D06P 5/20

(54) **METHOD FOR INKJET PRINTING OF A TEXTILE**
TINTENSTRAHLDRUCKVERFAHREN FÜR TEXTILIEN
PROCÉDÉ D'IMPRESSION TEXTILE PAR JET D'ENCRE

(30) Priority: 12.02.2002 US 356263 P
(43) Date of publication of application: 10.11.2004
(73) Proprietor: E.I. DU PONT DE NEMOURS AND COMPANY, Wilmington, Delaware 19898 (US)
(72) Inventor: BACCAY, Romeo, A., Acworth, GA 30102 (US); ANTON, Waifong, L., Wilmington, DE 19803 (US); RAYMOND, Michael, W., Newark, DE 19711 (US)
(74) Representative: Gritschneder, Martin
(86) International application number: PCT/US2003/004327
(87) International publication number: WO 2003/069054

(56) References cited:
- EP-A- 0 212 655
- WO-A-00/47422
- DE-A- 19 930 858
- DE-A- 19 930 986

## Description

### FIELD OF THE INVENTION

This invention pertains to a method for inkjet printing of textiles and the post treatment thereof for improved durability, in particular to post treatment with a combination of heat and pressure for improved crock-fastness.

### BACKGROUND OF THE INVENTION

The printing of textiles is currently accomplished primarily by rotary screen methods. In operation, screen printing is rapid and, for large runs, cost effective. However, cutting screens is expensive and time consuming thus making the per-unit cost for short runs quite substantial and, in many cases, prohibitive.

A digital printing method such as inkjet printing offers a number of potential benefits over conventional screen printing methods. Digital printing eliminates the set up expense associated with screen preparation and can potentially enable cost-effective short run production.

Inkjet printing furthermore allows visual effects such as tonal gradients and infinite pattern repeat size that cannot be practically achieved by a screen printing process.

One such digital printing system for textiles is disclosed in WO-03/029007 (Prior art according to Art. 54(3) EPC).

However, inkjet printing as it exists today is disadvantageous because of relatively slow speed. To be competitive with screen printing even for short runs, the speed of inkjet printers needs to increase.

Another disadvantage of inkjet printing, in particular inkjet printing with pigmented ink, is inkjet printed fabrics are particularly susceptible to color removal by abrasion and thus have poor durability or crock-fastness.

Even as inkjet hardware improvements are made to increase printing speeds, adoption of inkjet printing in the textile industry will be impeded if methods to also improve crock-fastness are not found.

US4597794 discloses inkjet ink formulations suitable for textile. Fabrics were imaged with this ink and set by heating at 150°C for five minutes. Wash-fastness was described as excellent.

US5897694 discloses inkjet ink formulations comprising, as an additive, a transition metal chelate, which provides improved wash-fastness.

US5958561 discloses an ink/textile combination wherein the textile is pretreated with a cross-linkable thermoplastic polymer and then imaged with an aqueous ink and cured at temperatures of 100-190°C. Improved wash-fastness was obtained.

US6146769 discloses an ink/textile combination wherein an interactive polymer, in the ink or pretreated or on the textile, helps bind the particulate colorant and provide wash-fastness.

US2002/0130939 describes a printer provided with a pressure/heater roller device for post processing of printer output, but primarily only addresses the mechanical aspects of post processing for paper print media.

Japanese laid open patent Hei 9-143407 discloses an inkjet ink with a thermoset resin which is imaged on fabric and fixed by heating at 130°C. The image is said to be water resistant.

Japanese laid open patent Hei 8-283636 discloses an inkjet ink with specified resin emulsions having high Tg. Fabric imaged with this ink is fixed at elevated temperature to provide wash-fastness.

DE-A 199 30 986 discloses in example 33 a method for inkjet printing of a textile, in which the printed textile is treated with a hot press or an iron. The ink is a reactive dye and the textile has DIN-A3-size. The fabric is covered by a sheet on the side opposit the printing head during printing in order to stabilize the textile material and to retain the ink on the textile.

### SUMMARY OF THE INVENTION

The invention as claimed in claim 1 solves the problem of how to improve the durability of injet images on textile and to provide inkjet printed textiles with good crock-fastness.

It was found that the crock-fastness of an inkjet-printed textile could be improved to a commercially acceptable level by fusion treating the printed textile with a combination of heat and pressure.

The fusion, in accordance with the present invention, can be performed in-line with the inkjet printer or performed separately, off-line.

The instant method improves the durability of textiles printed with pigmented inkjet inks, and allows the achievement of commercially acceptable durability for pigmented ink jet ink printed textiles. Thus, another aspect of the present invention is a textile printed with a pigmented ink, said printed textile having a dry crock-fastness of at least 4 and a wet crock-fastness of at least 3 (as measured in accordance with AATCC Test Method 8).

These and other features and advantages of the present invention will be more readily understood by those of ordinary skill in the art from a reading of the following detailed description.

### BRIEF DESCRIPTION OF THE DRAWINGS

Figure 1 depicts an embodiment of the present invention wherein the fusion of the inkjet-printed fabric is accomplished by treatment with heated nip rollers.
Figure 2 depicts another embodiment of the present invention wherein the fusion is accomplished by heating the inkjet printed fabric with a heated platen or a radiant heater, or a combination of the two, and immediately applying pressure to the warm fabric with nip rollers.
Figure 3 depicts a Glenro-type fuser wherein the printed textile is transported on a continuous belt through an oven-like heating zone to bring it up to fusion temperature; at the end of this zone the textile and the upper and lower belts are nipped with rollers such that pressure is applied to the heated textile.

### DETAILED DESCRIPTION OF THE PREFERRED EMBODIMENTS

The instant method is applicable to textiles printed with any inkjet printer. Suitable commercially available inkjet printers designed for textile include, for example, DuPont 3210 and 2020 Textile Printers (DuPont, Wilmington, DE), Textile Jet (Mimaki USA, Duluth, GA), DisplayMaker Fabrijet (MacDermid ColorSpan, Eden Prairie, MN), Amber, Zircon and Amethyst (Stork®) and the like.

The inkjet inks can be any inks suitable for textile, especially those suitable for jetting in the aforementioned and similar printers. Preferably, the inks are pigmented. Suitable inks also include those in the aforementioned references, such as in WO-03/029007. See also EP-A-1158029.

Pigment ink formulations for textiles will typically contain binder. Binders will preferably have a softening point (as indicated by glass transition temperature, Tg, or minimum film forming temperature, MFT) of less than about 60°C, more preferably less than about 30°C and even more preferably less than about 20°C. Binders with higher softening points tend to be harder to the touch and when incorporated in textile, cause the feel to be rough. The feel of a textile is referred to as the "hand". Generally, a softer hand is preferred.

Textiles useful in this invention include, but are not limited to cotton, wool, nylon, polyester and the like, and blends thereof. The finished form of the textile includes, but is not limited to, fabrics, garments, furnishings such as carpets and upholstery fabrics, and the like. Textiles can contain natural and synthetic materials, and blends thereof, and can be treated or untreated as is known in the art.

The printed textile is fused at elevated temperature and pressure. Upper temperature is dictated by the tolerance of the particular textile being printed. Lower temperature is determined by the amount of heat needed to achieve the desired level of durability. Generally, fusion temperatures will be at least about 80°C and preferably at least about 100°C, more preferably at least about 140°C and most preferably at least about 160°C.

Fusion pressures required to achieve improved crock can be very modest. Thus, pressures can be about 20.7 kPa (3 psi), preferably at least about 34.5 kPa (5 psi), more preferrable at least about 55.2 kPa (8 psi) and most preferably at least about 69 KPa (10 psi). Fusion pressures of about 207 kPa (30 psi) and above seem to provide no additional benefit to crock, but such pressures are not excluded.

The duration of fusion (amount of time the printed textile is under pressure at the desired temperature) was not found to be particularly critical. Most of the time in the fusion operation generally involves bringing the print up to the desired temperature. Once the print is fully up to temperature, the time under pressure can be brief (seconds).

Referring to Figure 1, there is depicted an embodiment wherein the fusion of the inkjet printed fabric is accomplished by treatment with heated nip rollers. The printed textile 2 is transported, under tension, over a heated roller 4 of sufficient diameter to provide adequate contact time at a given transport speed to allow temperatures reach desired levels. A second roller 6, covered with temperature resistant, pliant materials (e.g. silicone rubber), applies pressure to the heated print by nipping it against the heated roller 4.

Referring to Figure 2, there is depicted another embodiment wherein the fusion is accomplished by heating the inkjet printed fabric 10 with a heated platen 12 or a radiant heater 14, or a combination of the two, and immediately applying pressure to the warm fabric with nip rollers 16. The print is maintained at fusion temperature during application of pressure.

Referring to Figure 3, the printed textile 20 is transported on a continuous belt through an oven-like heating zone 24 to bring it up to fusion temperature; at the end of this zone the textile and the upper and lower belts are nipped with rollers 22 such that pressure is applied to the heated textile 28.

In yet another embodiment (not depicted) printed textile is placed, in a batch process, between two flat, parallel platens which are heated to fusing temperature and pressed together to achieve the desired fusion pressure.

The size of any fusion apparatus is dictated by the dimension of the fabric being treated. Typically fabric will be printed in rolls with widths of from 1 to 3 meters and thus the fusion zone of a fusion apparatus will preferably accommodate widths in that range.

From the viewpoint of commercial operation, the fusion operation is preferably performed in a continuous mode, although batch operation is also operable. The fuser can be positioned in-line with the inkjet printer such that the printed textile is fused immediately after printing. Alternatively, the fuser can be positioned off-line such that the printed textile is collected after printing and separately subjected to fusing.

With current technology, the fusing operation can be performed at faster rates than the textile can be inkjet-printed. Thus, an off-line fusing apparatus could potentially handle output from more than one inkjet printer. An in-line fusing apparatus would operate at the same rate as the printer.

### EXAMPLES

Inkjet printers and inks used in the following examples were 1) a DuPont Ink Jet 3210 printer and associated pigmented inks available under the Artistri™ tradename (P874 Cyan, P813 Magenta, P845 Yellow, P893 Black, P834 Orange, P869 Green); and, 2) an Epson Stylus® C80 printer and associated pigment inks available under the tradename Durabrite™ (T0323 magenta and T0322 cyan).

The fabrics used were obtained from Testfabrics, Inc., namely 1) 100% cotton fabric style # 419W which is a, bleached, mercerized combed broadcloth (133x72); and, 2) Polyester/cotton fabric, style # 7436M which is a 65/35 poplin, mercerized and bleached.

Two different fusing apparatus were employed: 1) a Glenro (Paterson, NJ) Bondtex™ Fabric and Apparel Fusing Press which moves the printed fabric between two heated belts equipped with adjustable pneumatic press and finally through a nip roller assembly; and, 2) a platen press, assembled for the purpose of precisely controlling temperature and pressure.

It should be noted that the Glenro Bondtex™ Fabric and Apparel Fusing Press is advertised for use in flatbed laminating of two or more layers of substrate materials. This operation of this unit, therefore, has been adapted for the fusion process of the present invention.

The platen press comprised of two parallel 6" square platens with embedded resistive heating elements that were set to maintain a desired platen temperature. The platens were fixed in a mutually parallel position to a pneumatic press that could press the platens together at a desired pressure by means of adjustable air pressure. Care was taken to be sure the platens were aligned so as to apply equal pressure across the entire work piece being fused. The effective area of the platen could be reduced, as needed, by inserting a spacer (made, for example from silicone rubber) of appropriate dimensions to allow operation on smaller work pieces.

Crock-fastness was determined according to the procedure described in AATCC Test Method 8 (Research Triangle Park, NC).

According to this method, a piece of test fabric supplied expressly for this evaluation is affixed to a 'finger' on the crocking device. The fabric-covered finger is then put in contact with the inkjet-printed textile, under prescribed pressure, and driven repetitively across the fabric a prescribed number of times. Crock is assessed by measuring the amount of color transferred from the printed sample to the test fabric. Measurement can be done visually by estimating the color transfer compared to a standard AATCC scale. Measurement can also be done instrumentally with a spectrophotometer, for example a Minolta Spectrophotometer CM-3600d interfaced with SpectraMatch Version (V.3.3.5 D) and Color Sensor (version: 203,13011028) software from CyberChrome, Inc.

Two crock measurements were taken, one with dry test fabric (called Dry Crock) and one with the test fabric moistened with de-ionized water (called Wet Crock).

A crock rating scale of 1 to 5 was applied, wherein 5 denotes negligible or no change, 4 denotes slightly changed, 3 denotes noticeably changed, 2 denotes considerably changed, and 1 denotes much change in color. A difference of 0.5 units is considered significant and would be evident to most observers.

Commercially acceptable minimum values are generally considered to be 4 for dry crock and 3 for wet crock.

### Example 1

This example demonstrates the improved crock-fastness obtained for samples of Artistri™ ink, printed on the DuPont printer at 100% coverage (about 15 grams, wet weight, of ink per square meter of fabric) and fused with the Glenro press. The press was operated with the top and bottom rollers set for a temperature of 180°C (actual temperature achieved on fabric surface cannot be determined), nip rollers set point for a pressure of 620.5 kPa (90 psia), (actual pressure achieved on fabric surface could not be accurately determined) a web speed of 0.9 m/mm of (3 ft/min) and a dwell time of 53 seconds in the heating/treatment area.

Table 1 provides crock values (visual estimation) for inventive samples compared to ambient drying and to drying in an oven at 140°C for 30 minutes (no pressure). Fabric was 419W cotton.

**Table 1**

| | Dry Crock | | | Wet Crock | | |
|---|---|---|---|---|---|---|
| Artistri Inks | Ambient Drying | Oven Drying | Fusing Press | No Drying | Oven Drying | Fusing Press |
| Cyan | 3.0 | 4.0 | 4.5 | 1.5 | 3.0 | 3.0 |
| Magenta | 3.0 | 3.5 | 4.5 | 1.5 | 3.0 | 3.0 |
| Yellow | 3.0 | 3.0 | 4.5 | 1.5 | 2.5 | 2.5 |
| Black | 2.5 | 2.5 | 4.5 | 1.5 | 2.5 | 2.5 |
| Orange | 3.0 | 3.0 | 4.0 | 1.5 | 2.5 | 3.0 |
| Green | 4.5 | 3.0 | 5.0 | 2.5 | 3.5 | 3.5 |

Results indicate that application of fusion substantially improves dry crock over heating alone or no heat at all. For wet crock, similar improvement over ambient drying is obtained for either oven drying or fusion. However, oven drying would be impracticably slow for commercial purposes.

### Example 2

This example demonstrates the improved crock-fastness obtained for samples of Artistri™ cyan ink, printed on the DuPont printer (100% coverage) and fused with the platen press. All crock measurements were spectrophotometric.

Table 2A provides crock values for inventive samples fused at the indicated temperatures, pressures, and duration compared to control samples allowed to dry under ambient conditions (no heat, no pressure, four replicates). Application of fusion improves crock. There was little sensitivity to the range of fusing pressures, 206.8-620.5 KPa (30-90 psi), and durations, 30-90 seconds, studied.

**Table 2A**

| | Fusion | | | 419W cotton | | 7436M cotton/poly | |
|---|---|---|---|---|---|---|---|
| Trial | Temp. (°C) | Pres.* (psi) | Duration (sec) | Dry Crock | Wet Crock | Dry Crock | Wet Crock |
| 1 | 140 | 30 | 90 | 3.89 | 2.61 | 4.3 | 3.2 |
| 2 | 140 | 70 | 90 | 4.63 | 2.65 | 4.07 | 2.76 |
| 3 | 140 | 50 | 60 | 4.53 | 2.63 | 4.22 | 2.82 |
| 4 | 140 | 30 | 30 | 4.4 | 2.54 | 3.72 | 2.62 |
| 5 | 140 | 70 | 30 | 4.39 | 2.48 | 4.26 | 3.13 |
| 6 | 160 | 30 | 60 | 4.29 | 2.5 | 4.19 | 2.9 |
| 7 | 160 | 50 | 60 | 4.34 | 2.89 | 4.24 | 3.27 |
| 8 | 160 | 50 | 30 | 4.53 | 2.64 | 4.32 | 2.97 |
| 9 | 160 | 50 | 90 | 4.51 | 2.68 | 4.16 | 3.07 |
| 10 | 160 | 70 | 60 | 4.69 | 3 | 4.67 | 3.43 |
| 11 | 180 | 30 | 90 | 4.32 | 2.78 | 4.01 | 3.17 |
| 12 | 180 | 30 | 30 | 4.25 | 3.05 | 4.32 | 2.96 |
| 13 | 160 | 50 | 60 | 4.36 | 2.66 | 4.39 | 3.01 |
| 14 | 180 | 50 | 60 | 4.54 | 2.99 | 4.45 | 2.94 |
| 15 | 180 | 70 | 90 | 4.69 | 2.77 | 4.65 | 3.24 |
| 16 | 180 | 70 | 30 | 4.69 | 3.01 | 4.48 | 3.35 |
| Control 1 | 0 | 0 | 0 | 4.2 | 1.79 | 2.95 | 2.2 |
| Control 2 | 0 | 0 | 0 | 4.32 | 1.8 | 3.35 | 1.82 |
| Control 3 | 0 | 0 | 0 | 3.17 | 1.56 | 3.36 | 1.86 |
| Control 4 | 0 | 0 | 0 | 3.11 | 1.48 | 2.72 | 1.7 |

| | | | | | | | |
|---|---|---|---|---|---|---|---|
| * 30 psi ≙ 206.8 kPa; 50 psi ≙ 344.7 kPa; 70 psi ≙ 482.6 kPa. | | | | | | | |

Table 2B provides crock values for inventive samples fused at the indicated temperatures, pressures, and duration compared to control samples which a) were air dried then subjected to the indicated pressure and b) were oven dried at 160°C for 30 min then cooled and subjected to pressure. Fabric was 419W cotton.

**Table 2B**

| Pressure | No heat-pressure only | | Oven (160°C/30min.) then cooled, then pressure | | Fusion (160°C and pressure for 60 sec.) | |
|---|---|---|---|---|---|---|
| (psi)* | dry crock | wet crock | dry crock | Wet crock | dry crock | wet crock |
| 60 | 4.36 | 1.92 | 3.91 | 2.95 | 4.57 | 2.87 |
| 50 | 2.53 | 1.86 | 3.04 | 2.97 | 4.56 | 2.88 |
| 40 | 3.92 | 1.84 | 2.78 | 3.12 | 4.64 | 2.77 |
| 30 | 2.5 | 1.84 | 2.59 | 2.98 | 4.55 | 2.9 |
| 20 | 2.53 | 1.73 | 2.5 | 3.05 | 4.34 | 2.88 |
| 15 | 2.56 | 1.68 | 2.6 | 3.06 | 4.56 | 2.91 |
| 10 | 2.33 | 1.82 | 2.72 | 3.04 | 4.26 | 2.83 |
| 5 | 2.67 | 1.77 | 3.61 | 3.32 | 4.46 | 2.95 |
| 0 | 3.68 | 1.74 | 4.35 | 3.22 | --- | --- |

| | | | | | | |
|---|---|---|---|---|---|---|
| * 5 psi ≙ 34.5 kPa; 10 psi ≙ 68.95 kpa; 15 psi ≙ 103.5 kPa; 20 psi ≙ 137.9 kPa; 30 psi ≙ 206.85 kPa; 40 psi ≙ 275.8 kPa; 50 psi ≙ 345 kPa; 60 psi = 413.7 kPa. | | | | | | |

As can be seen from the results, application of fusion yields higher crock values compared to the control samples. Fusion pressures as low as 34.5 KPa (5 psi) are effective.

There tends to be substantial variability in dry crock results when samples are not fused (witness the control samples). Each crock value is the result of only one test. Variation is attributed mostly to actual differences in the fabric, rather than the test method itself. Fusing not only improves crock, but also tends to reduce sample-to-sample variation.

Table 2C provides crock values for inventive samples fused 160°C and 10 psi for 60 seconds. The time between printing and fusion was varied between 1 and 93 hours.

**Table 2C**

| Time between printing and fusion | Dry Crock | Wet Crock |
|---|---|---|
| 1 hour | 3.93 | 3.01 |
| 2 hours | 3.51 | 3.13 |
| 3 hours | 4.44 | 2.84 |
| 4 hours | 3.88 | 2.8 |
| 5 hours | 4.46 | 2.85 |
| 21 hours | 4.28 | 2.91 |
| 22 hours | 4.38 | 2.87 |
| 23 hours | 4.21 | 2.86 |
| 24 hours | 4.34 | 2.89 |
| 25 hours | 4.4 | 2.84 |
| 26 hours | 4.44 | 2.98 |
| 27 hours | 4.47 | 3.02 |
| 28 hours | 4.27 | 3.04 |
| 29 hours | 4.53 | 3.07 |
| 93 hours | 4.29 | 2.91 |

Results show that the high crock values (which come from fusion) can be achieved whether fusion is performed immediately after printing (such as an in-line operation) or days later (such as off-line operation).

### Example 3

This example demonstrates the improved crock-fastness obtained for samples of Durabrite™ cyan and magenta ink, printed on an Epson Stylus® C80 printer (100% coverage) and fused with the platen press. This ink and printer are designed for paper and not, per se, for textile. The textile had to be mounted on a substrate to enable transport through the printer.

Results, given in Table 3, show improved crock (spectrophotometric measurement) after fusing, although the magnitude of improvement is less than for previous examples that used ink specifically designed for textile.

**Table 3**

| | Fusion: 60 seconds at | | Epson cyan | | Epson magenta | |
|---|---|---|---|---|---|---|
| Fabric | °C | Psi* | dry crock | wet crock | dry crock | Wet crock |
| 419W cotton | No heat | 0 | 3.22 | 1.9 | 2.95 | 1.78 |
| | 140 | 50 | 3.2 | 2.07 | 2.86 | 1.68 |
| | 160 | 50 | 3.09 | 1.96 | 2.75 | 1.69 |
| | 160 | 50 | 3.11 | 2.03 | 2.85 | 1.71 |
| | 180 | 50 | 3.43 | 2.31 | 2.94 | 1.73 |
| 7436M poly/cotton | No heat | 0 | 2.57 | 1.75 | 2.38 | 1.62 |
| | 140 | 50 | 3.14 | 2.07 | 2.76 | 1.77 |
| | 160 | 50 | 3.1 | 2.05 | 2.79 | 1.76 |
| | 160 | 50 | 3.09 | 2.05 | 2.83 | 1.84 |
| | 180 | 50 | 3.3 | 2.28 | 2.84 | 1.89 |

| | | | | | | |
|---|---|---|---|---|---|---|
| * 50 psi ≙ 345 kPa | | | | | | |

## Claims

1. A method for inkjet printing of a textile, the method comprising the step of inkjet printing an ink jet ink onto a textile substrate and applying heat and pressure to produce an inkjet-printed textile, **characterized in that**
the fabric is printed in rolls with widths of from 1 to 3 m;
the inkjet-printed textile is printed with a pigmented inkjet ink; and
the inkjet-printed textile is treated with a fusing operation by the application of a combination of heat and pressure.

2. The method of claim 1, **characterized in that** the heat and pressure are applied simultaneously.

3. The method of claim 1, **characterized in that** heat is applied followed by the application of pressure.

4. The method of claim 1, **characterized in that** heat is applied at temperatures of at least about 80°C, and at least about 20.7 kPa (3 psi) of pressure is applied.

5. The method of claim 1, **characterized in that** the fusing operation is in-line with an inkjet printer producing the inkjet-printed textile such that fusing is effected in a continuous mode as the textile is printed.

6. The method of claim 1, **characterized in that** the fusing operation is off-line such that the inkjet-printed textile is collected after printing and separately subjected to fusing.

7. The method of claim 1, **characterized in that** the heat and pressure are applied simultaneously, heat is applied at temperatures of at least about 80°C, and at least about 20.7 kPa (3 psi) of pressure is applied.

8. The method of claim 1, **characterized in that** heat is applied followed by the application of pressure, heat is applied at temperatures of at least about 80°C, and at least about 20.7 kPa (3 psi) of pressure is applied.

## Patentansprüche

1. Verfahren zum Tintenstrahldrucken eines Stoffes, wobei das Verfahren den Schritt des Tintenstrahldruckens einer Tintenstrahltinte auf ein Stoffsubstrat und des Anwendens von Wärme und Druck umfaßt, um einen tintenstrahlbedruckten Stoff zu erzeugen, **dadurch gekennzeichnet, daß**
das Gewebe in Rollen mit Breiten von 1 bis 3 m bedruckt wird;
der tintenstrahlbedruckte Stoff mit einer pigmentierten Tintenstrahltinte bedruckt wird; und
der tintenstrahlbedruckte Stoff mit einem fixierenden Arbeitsgang durch die Anwendung einer Kombination von Wärme und Druck behandelt wird.

2. Verfahren nach Anspruch 1, **dadurch gekennzeichnet, daß** die Wärme und der Druck gleichzeitig angewendet werden.

3. Verfahren nach Anspruch 1, **dadurch gekennzeichnet, daß** Wärme angewendet wird und nachfolgend Druck angewendet wird.

4. Verfahren nach Anspruch 1, **dadurch gekennzeichnet, daß** Wärme mit Temperaturen von mindestens etwa 80°C angewendet wird und mindestens etwa 20,7 kPa (3 psi) Druck angewendet werden.

5. Verfahren nach Anspruch 1, **dadurch gekennzeichnet, daß** der fixierende Arbeitsgang in einer Anlage mit einem Tintenstrahldrucker ist, der den tintenstrahlbedruckten Stoff erzeugt, derart, daß Fixieren in einer kontinuierlichen Weise bewirkt wird, wenn der Stoff bedruckt wird.

6. Verfahren nach Anspruch 1, **dadurch gekennzeichnet, daß** der fixierende Arbeitsgang außerhalb einer Anlage ist, derart, daß der tintenstrahlbedruckte Stoff nach dem Drucken gesammelt und gesondert dem Fixieren unterworfen wird.

7. Verfahren nach Anspruch 1, **dadurch gekennzeichnet, daß** die Wärme und der Druck gleichzeitig angewendet werden, Wärme mit Temperaturen von mindestens etwa 80°C angewendet wird und mindestens etwa 20,7 kPa (3 psi) Druck angewendet werden.

8. Verfahren nach Anspruch 1, **dadurch gekennzeichnet, daß** Wärme angewendet wird, nachfolgend Druck angewendet wird, Wärme mit Temperaturen von mindestens etwa 80°C angewendet wird und mindestens etwa 20,7 kPa (3psi) Druck angewendet werden.

## Revendications

1. Procédé d'impression textile par jet d'encre, le procédé comprenant l'étape d'impression par jet d'encre d'une encre pour jet d'encre sur un substrat textile, et l'application d'une chaleur et d'une pression pour produire un textile imprimé par jet d'encre, **caractérisé en ce que**:
le tissu est imprimé en rouleaux d'une largeur de 1 m à 3 m;
le textile imprimé par jet d'encre est imprimé avec une encre pour jet d'encre pigmentée; et
le textile imprimé par jet d'encre est traité avec une opération de fusion par l'application d'une combinaison de chaleur et de pression.

2. Procédé selon la revendication 1, **caractérisé en ce que** la chaleur et la pression sont appliquées simultanément.

3. Procédé selon la revendication 1, **caractérisé en ce que** la chaleur est d'abord appliquée, suivie par l'application de la pression.

4. Procédé selon la revendication 1, **caractérisé en ce que** la chaleur est appliquée à des températures d'au moins environ 80°C, et une pression d'au moins environ 20,7 kPa (3 psi) est appliquée.

5. Procédé selon la revendication 1, **caractérisé en ce que** l'opération de fusion est exécutée en ligne avec une imprimante à jet d'encre produisant le textile imprimé par jet d'encre de telle sorte que la fusion soit exécutée dans un mode continu pendant que le textile est imprimé.

6. Procédé selon la revendication 1, **caractérisé en ce que** l'opération de fusion n'est pas exécutée en ligne, de telle sorte que le textile imprimé par jet d'encre soit récupéré après l'impression et soit soumis séparément à la fusion.

7. Procédé selon la revendication 1, **caractérisé en ce que** la chaleur et la pression sont appliquées simultanément, la chaleur est appliquée à des températures d'au moins environ 80°C, et une pression d'au moins environ 20,7 kPa (3 psi) est appliquée.

8. Procédé selon la revendication 1, **caractérisé en ce que** la chaleur est d'abord appliquée, suivie par l'application de la pression, la chaleur est appliquée à des températures d'au moins environ 80°C, et une pression d'au moins environ 20,7 kPa (3 psi) est appliquée.
